

# United States Patent

Ito et al.

[15] 3,652,267

[45] Mar. 28, 1972

[54] **CARBON STEELS AND ALLOY STEELS  
FOR COLD FORGING**

- [72] Inventors: **Tetsuro Ito; Azuma Hiki**, both of Nagoya, Aichi, Japan
- [73] Assignee: **Daido Seiko Kabushiki Kaisha**, Aichi Prefecture, Japan
- [22] Filed: **Sept. 23, 1968**
- [21] Appl. No.: **761,463**

[30] **Foreign Application Priority Data**

Oct. 11, 1967 Japan.....42/64954

- [52] U.S. Cl.....75/123 L, 75/123 R, 75/126 G  
[51] Int. Cl.....C22c 39/00  
[58] Field of Search.....75/58, 123, 129, 123 L, 123 R

[56]

**References Cited**

**UNITED STATES PATENTS**

|           |         |                |          |
|-----------|---------|----------------|----------|
| 3,000,731 | 9/1961  | Ototani.....   | 75/129   |
| 3,212,881 | 10/1965 | Dunn .....     | 75/58 X  |
| 3,215,525 | 11/1965 | Sprankle ..... | 75/58 X  |
| 3,275,433 | 9/1966  | Hilty .....    | 75/58 X  |
| 3,309,194 | 3/1967  | Dunn .....     | 75/58 X  |
| 2,258,604 | 10/1941 | Gagnebin.....  | 75/123 X |

*Primary Examiner*—L. Dewayne Rutledge

*Assistant Examiner*—Joseph E. Legru

*Attorney*—Wenderoth, Lind & Ponack

[57]

**ABSTRACT**

This invention relates to machine structural carbon steels and alloy steels having an excellent cold forging property. Such a steel can be produced by deoxidizing a carbon steel or an alloy steel with a calcium-silicon alloy and controlling the calcium content thereof.

**6 Claims, 3 Drawing Figures**

PATENTED MAR 28 1972

3,652,267



FIG.1



FIG.2



FIG.3

INVENTORS  
TETSURO ITO  
AZUMA HIKI

BY *Wendorff, Hind & Snack*  
ATTORNEYS

### CARBON STEELS AND ALLOY STEELS FOR COLD FORGING

This invention relates to machine structural carbon steels and alloy steels which can be cold forged and are produced by deoxidizing carbon steels and alloy steels with a calcium-silicon alloy. Particularly, this invention relates to machine structural carbon steels and alloy steels having an excellent cold forging property and containing calcium in an amount varying from 0.0015 percent to 0.0060 percent by weight.

Heretofore, it was reported by H. Opitz and others that the machine structural carbon steel designated as S45C steel becomes to have a better machinability after it was deoxidized by using a calcium-silicon alloy such as Ca<sub>2</sub>Si or CaSi<sub>2</sub> than that of the S45C steel which was deoxidized by using aluminium or silicon. Also it was reported by Hasegawa and others that stainless steels become to have good hot workability after they were deoxidized by using a calcium alloy.

In the course of the investigation for improving the machinability of the machine structural carbon steels and alloy steels, we have found the new fact that their cold forging property is remarkably improved when they are deoxidized by using a calcium-silicon alloy such as Ca<sub>2</sub>Si or CaSi<sub>2</sub> and the calcium content retained therein is controlled to the range varying from 0.0015 percent to 0.0060 percent by weight.

This invention is fully explained by referring to the accompanying drawings in which:

FIG. 1 shows a curve illustrating the relationship between the calcium content and the critical reduction in height for initiating the visible surface crack of machine structural carbon steel designated as S45C steel in the Japanese Industrial Standards after it was deoxidized by using a calcium-silicon alloy which contains calcium in an amount varying from 30 percent to 35 percent by weight and silicon in an amount varying from 55 percent to 65 percent by weight. It is noted that the critical reduction in height is calculated by the following equation.

$$\frac{H_0 - H}{H_0} \times 100 (\%)$$

wherein H<sub>0</sub> indicates the initial height of the test piece and H indicates the final height of the test piece after it was compressed. The test piece has the size of 6mm. in diameter and 12mm. in height, and it was polished with a grinder. The test piece was compressed at the speed of 5mm. per minute. The test was conducted for 20 test pieces and the critical reduction in height is given as the average value.

As it is obvious from FIG. 1, the maximum value of the critical reduction in height is obtained at the point indicating the calcium content of 0.0025 percent by weight.

FIG. 2 shows two curves illustrating the critical reduction in

steels were deoxidized by using the aluminum. The same pieces as in FIG. 1 were made and the test pieces were subjected to the thermal treatment for spheroidizing annealing them and then they were tested for the critical reduction in height in the same manner as in FIG. 1. It is obvious from the curves (I) and (II) as shown in FIG. 2 that the steels which were deoxidized with the calcium alloy have better cold forging property than that of the steels which were deoxidized with aluminum.

FIG. 3 shows a curve illustrating the critical reduction in height of machine structural alloy steel designated as SCM3 steel in the Japanese Industrial Standards after it was deoxidized by using the calcium-silicon alloy as in FIG. 1 and the calcium content retained therein was controlled to 0.0025 percent by weight and also the steel was deoxidized by using the metallic aluminum and the aluminum content retained therein was controlled to 0.019 percent by weight, and then each steel was tested for the critical reduction in height in the same manner as in FIG. 1. It is obvious from the curve as shown in FIG. 3 that the steel which was deoxidized with the calcium-silicon alloy has better cold forging property than that of the steel which was deoxidized with aluminum in spite of the presence of the alloying components such as Cr and Mo.

Examples of the cold forging carbon steels and alloy steels achieved in accordance with this invention and the control examples are summarized in the following Table.

The various steels referred to in the present application are designated according to the Japanese Industrial Standards and are cold forgeable carbon steels having the following compositions:

S10C steel: 0.08 to 0.13 percent carbon, 0.15 to 0.35 percent silicon, 0.30 to 0.60 percent manganese and the balance being substantial iron and incidental impurities.

S20C steel: 0.18 to 0.23 percent carbon, 0.15 to 0.35 percent silicon, 0.30 to 0.60 percent manganese and the balance being substantially iron and incidental impurities.

S30C steel: 0.27 to 0.33 percent carbon, 0.15 to 0.35 percent silicon, 0.60 to 0.90 percent manganese and the balance being iron and incidental impurities.

S45C steel: 0.42 to 0.48 percent carbon, 0.15 to 0.35 percent silicon, 0.60 to 0.90 percent manganese and the balance being iron and incidental impurities.

S55C steel: 0.52 to 0.58 percent carbon, 0.15 to 0.35 percent silicon, 0.60 to 0.90 percent manganese and the balance being iron and incidental impurities.

SCM3 steel: 0.33 to 0.38 percent carbon, 0.15 to 0.35 percent silicon, 0.60 to 0.85 percent manganese, 0.90 to 1.20 percent chromium, 0.15 to 0.30 percent molybdenum, and the balance being substantially iron and incidental impurities.

| Steels                          | Chemical component |      |      |       |       |       |       |        |       |
|---------------------------------|--------------------|------|------|-------|-------|-------|-------|--------|-------|
|                                 | C                  | Si   | Mn   | P     | S     | Cr    | Mo    | Ca     | Al    |
| S10C deoxidized with a Ca-alloy | 0.11               | 0.31 | 0.48 | 0.018 | 0.016 | ..... | ..... | 0.0026 | ..... |
| S10C deoxidized with aluminium  | 0.09               | 0.29 | 0.52 | 0.020 | 0.013 | ..... | ..... | 0.0007 | 0.015 |
| S20C deoxidized with a Ca-alloy | 0.22               | 0.33 | 0.40 | 0.014 | 0.017 | ..... | ..... | 0.0022 | ..... |
| S20C deoxidized with aluminium  | 0.22               | 0.24 | 0.43 | 0.016 | 0.018 | ..... | ..... | 0.0006 | 0.014 |
| S30C deoxidized with a Ca-alloy | 0.32               | 0.32 | 0.70 | 0.013 | 0.019 | ..... | ..... | 0.0027 | ..... |
| S30C deoxidized with aluminium  | 0.29               | 0.30 | 0.71 | 0.019 | 0.029 | ..... | ..... | 0.0001 | 0.016 |
| S45C deoxidized with a Ca-alloy | 0.43               | 0.28 | 0.73 | 0.019 | 0.005 | ..... | ..... | 0.0025 | ..... |
| S45C deoxidized with aluminium  | 0.43               | 0.31 | 0.71 | 0.019 | 0.012 | ..... | ..... | 0.0009 | 0.013 |
| S55C deoxidized with a Ca-alloy | 0.56               | 0.25 | 0.78 | 0.014 | 0.016 | ..... | ..... | 0.0028 | ..... |
| S55C deoxidized with aluminium  | 0.54               | 0.29 | 0.72 | 0.018 | 0.017 | ..... | ..... | 0.0001 | 0.014 |
| SCM3 deoxidized with a Ca-alloy | 0.36               | 0.31 | 9.75 | 0.014 | 0.014 | 1.94  | 0.23  | 0.0025 | ..... |
| SCM3 deoxidized with aluminium  | 0.35               | 0.28 | 0.71 | 9.017 | 0.011 | 1.01  | 0.21  | 0.0001 | 0.019 |

height for initiating the visible surface crack of machine structural carbon steels designated as S10C steel, S20C steel, S30C steel, S45C steel and S55C steel in the Japanese Industrial Standards after they were deoxidized by using a calcium alloy or aluminum and the calcium or aluminum content retained in them was controlled to an amount varying from 0.0022% Ca to Al % Ca by weight or from 0.016% al. to 0.028% Al by weight. The curve (I) shows the critical reduction in height when the above-mentioned steels were deoxidized by using the calcium-silicon alloy as in FIG. 1 and the curve (II) shows the critical reduction in height when the above-mentioned

65

70

75

We claim:

1. A cold forgeable carbon steel, characterized in that a steel consisting essentially of 0.08 to 0.13 percent of carbon 0.15 to 0.35 percent of silicon, 0.30 to 0.60 percent of manganese and the balance substantially iron and incidental impurities is deoxidized with a calcium-silicon alloy and controlled so as to contain calcium in an amount varying from 0.0015 to 0.0060 percent.

2. A cold forgeable carbon steel, characterized in that a steel consisting essentially of 0.18 to 0.23 percent of carbon, 0.15 to 0.35 percent of silicon, 0.30 to 0.60 percent of man-

ganese and the balance substantially iron and incidental impurities is deoxidized with a calcium-silicon alloy and controlled so as to contain calcium in an amount varying from 0.0015 to 0.0060 percent.

3. A cold forgeable carbon steel, characterized in that a steel consisting essentially of 0.27 to 0.33 percent of carbon, 0.15 to 0.35 percent of silicon, 0.60 to 90 percent of manganese and the balance substantially iron and incidental impurities is deoxidized with a calcium-silicon alloy and controlled so as to contain calcium in an amount varying from 0.0015 to 0.0060 percent.

4. A cold forgeable carbon steel, characterized in that a steel containing 0.42 to 0.48 percent of carbon, 0.15 to 0.35 percent of silicon, 0.60 to 0.90 percent of manganese and the balance substantially iron and incidental impurities is deoxidized with a calcium-silicon alloy and controlled so as to contain calcium in an amount varying from 0.0015 to 0.0060 percent.

5. A cold forgeable carbon steel, characterized in that a steel consisting essentially of 0.52 to 0.58 percent of carbon, 0.15 to 0.35 percent of silicon, 0.60 to 0.90 percent of manganese and the balance substantially iron and incidental impurities is deoxidized with a calcium-silicon alloy and controlled so as to contain calcium in an amount varying from 0.0015 to 0.0060 percent.

6. A cold forgeable Cr-Mo base steel, characterized in that a steel consisting essentially of 0.33 to 0.38 percent of carbon, 0.15 to 0.35 percent of silicon, 0.60 to 0.85 percent of manganese, 0.90 to 1.20 percent of chromium, 0.15 to 0.30 percent of molybdenum and the balance substantially iron and incidental impurities is deoxidized with a calcium-silicon alloy and controlled so as to contain calcium in an amount varying from 0.0015 to 0.0060 percent.

\* \* \* \* \*

20

25

30

35

40

45

50

55

60

65

70

75